

# UNITED STATES PATENT OFFICE.

OLIVER B. McMILLIN, OF PITTSBURGH, PENNSYLVANIA, ASSIGNOR, BY MESNE ASSIGNMENTS, TO PITTSBURGH ROLLS CORPORATION, OF PITTSBURGH, PENNSYLVANIA, A CORPORATION OF VIRGINIA.

## ALLOY OF IRON.

1,252,596.

Specification of Letters Patent. Patented Jan. 8, 1918.

No Drawing. Application filed July 29, 1916, Serial No. 112,074. Renewed May 26, 1917. Serial No. 171,293.

To all whom it may concern:

Be it known that I, OLIVER B. McMILLIN, a citizen of the United States, residing at Pittsburgh, in the county of Allegheny and State of Pennsylvania, have invented 5 certain new and useful Improvements in Alloys of Iron, of which the following is a specification.

My invention relates to an alloy of iron, 10 and particularly one in which a high proportion of sulfur is used.

The element sulfur is ordinarily considered a deleterious or weakening element; 15 but I have found that when proportionately combined with the several other elements comprising the present invention, the presence of sulfur in higher proportions than those customarily used, and ordinarily considered objectionable, is not only not harmful, but adds appreciably to the beneficial 20 result of the entire mixture.

In carrying out my invention, I mix with iron, either in an air furnace or open hearth furnace, or in a cupola or any other suitable heating furnace, proportions of silicon, 25 sulfur, phosphorus, manganese and chromium, as hereinafter stated, together with a content of total carbon, within the ranges stated.

30 Suitable proportions of these several metallic elements are as follows, it being understood that minimum and maximum proportions are given in percentages, and that the remaining quantum of material to make 35 up the entire 100% is ordinary gray or foundry iron or scrap metal:

|                   |                |
|-------------------|----------------|
| Silicon -----     | .25% to 1.00%  |
| Sulfur -----      | .05% to 2.00%  |
| Phosphorus -----  | .05% to 2.00%  |
| Manganese -----   | .20% to 1.00%  |
| Chromium -----    | .25% to 3.00%  |
| Total carbon----- | 1.50% to 3.50% |

The alloy within the above stated proportions is particularly adapted for the making 45 of plate mill rolls, sheet mill rolls, tin plate rolls, and other rolls or similar articles requiring a hard, resisting, dense surface of

considerable depth, adapted to resist abrasion and wear. 50

The especial quality of the sulfur content is that it increases the depth of chill in proportion to the amount of sulfur used, especially in combination with the accompanying content of chromium. 55

The percentages of the alloying metals may be varied within the minimum and maximum limits above given, according to the desired result. Thus I have secured excellent results in the manufacture of rolls 60 with a preferred mixture made as follows:

|                   |        |
|-------------------|--------|
| Silicon -----     | .50%   |
| Sulfur -----      | .12%   |
| Phosphorus -----  | .08%   |
| Manganese -----   | .30%   |
| Chromium -----    | 1.00%  |
| Total carbon----- | 2.40%  |
| Iron -----        | 95.60% |

The alloying elements react and combine 70 upon and with each other, producing the metallurgical results, molecular changes, and resulting effects desired, avoiding undue brittleness, and producing in the resulting casting a characteristic hard, dense, and 75 deeply penetrating outer body portion for the roll, hammer die, anvil, or other article into which the mixture is formed.

Having described my invention, what I claim is:

1. An alloy composed of iron combined with silicon ranging from .25% to 1.00%, chromium from .25% to 3.00%, sulfur .05% to 2.00%, phosphorus .05% to 2.00%, manganese .20% to 1.00%, total carbon 1.50% 85 to 3.50%.

2. An alloy composed of silicon .50%, sulfur .12%, phosphorus .08%, manganese .30%, chromium 1.00%, total carbon 2.40% and iron 95.60%. 90

In testimony whereof I hereunto affix my signature in the presence of two witnesses.

OLIVER B. McMILLIN.

Witnesses:

C. M. CLARKE,  
W. A. HECKMAN.